

# United States Patent Office.

JOEL PUTNAM, OF DANVERS, MASSACHUSETTS.

*Letters Patent No. 93,002, dated July 27, 1869.*

## IMPROVEMENT IN FINISHING SPLIT LEATHER.

The Schedule referred to in these Letters Patent and making part of the same.

*To all persons to whom these presents may come:*

Be it known that I, JOEL PUTNAM, of Danvers, of the county of Essex, and State of Massachusetts, have made a new and useful invention or improvement having reference to the Finishing of Split Leather; and do hereby declare the same to be described as follows:

My improvement imparts to the inner side or surface of a piece of split leather an appearance closely resembling that of the hair-side of what is termed "kip leather." It not only does this, but renders the leather better for the manufacture of shoes or other articles, as well as for use afterwards when so made up, as it prevents the leather from discoloring the feet or stockings of the wearer of the shoe, and causes it to be softer and more pliable, as well as a better resister of moisture or water.

In carrying out my invention, I first make a composition, which may be composed of one pound of glue, one-half pint of boiled linseed-oil, and about one-half an ounce of vermillion, or other suitable pigment.

The glue should be dissolved in hot or boiling water, so as to make a solution of the consistency of such as is commonly used for cementing wood, afterwards the

oil and the pigment should be thoroughly incorporated or mixed with the solution of glue.

The composition thus made is next to be applied to the surface of the piece of leather by means of a brush, two or any other suitable number of coatings being so laid on, and each being allowed to become dry before application of the next one.

After the application of each coating, it should be "glossed" by a currier's "glassing-tool."

Finally, the leather so coated should be boarded, this process, as well as that of glassing it, being well understood by curriers.

I claim as my invention, the above-described method of preparing the surface of split leather, the same consisting in applying thereto a composition substantially as set forth, and glassing and boarding it.

I also claim the improved manufacture of split leather as so made or treated.

JOEL PUTNAM.

Witnesses:

R. H. EDDY,  
S. N. PIPER.